

# UNITED STATES PATENT OFFICE.

THOMAS SOTTILE, OF UNION, NEW JERSEY.

## COMPOSITION OF MATTER.

1,024,156.

Specification of Letters Patent. Patented Apr. 23, 1912.

No Drawing.

Application filed September 12, 1911. Serial No. 648,971.

*To all whom it may concern:*

Be it known that I, THOMAS SOTTILE, a subject of Italy, residing at 172 Palisade avenue, town of Union, in the county of Hudson and State of New Jersey, Weehawken P. O., New Jersey, have invented a new and useful Composition of Matter to be Used on Razor-Strrops for Sharpening Razors for Shaving Purposes, of which the

10 following is a specification:

This invention relates to a new and useful composition of matter adapted to be applied to razor strops.

15 My improved composition consists of the following ingredients combined in the proportions stated, viz:

|                        |                      |
|------------------------|----------------------|
| Water                  | Half glass.          |
| Powdered steel         | Two pounds.          |
| 20 Axe grease          | One and half pounds. |
| Powdered glass         | Small quantity.      |
| Anisette oil (perfume) | Small quantity.      |

These ingredients are to be thoroughly mingled by agitation.

25 By using the above-named composition on the razor strop it will give the razor a keen edge. By the use of the above composition

by stropping the razor is always ready for shaving.

I am aware that a certain composition 30 consisting of powdered emery and paste has been used and patented for the same purposes, but I am not aware that all the ingredients of my composition have been used together.

35

I claim:

1. The herein-described composition of matter, consisting of water, powdered steel, axle grease, powdered glass, and anisette oil, substantially as described and for the purpose specified.

2. The herein-described composition of matter on razor strops, for sharpening razors for shaving, consisting of water, half glass; powdered steel, two pounds; axle 45 grease, one and half pounds; powdered glass, small quantity; anisette oil, small quantity (perfume), substantially as described.

THOMAS SOTTILE.

Witnesses:

JOHN STEIN,  
JOE KREMIN.